

## UNITED STATES PATENT OFFICE

2,488,891

METHOD OF MAKING ABRASIVE GRINDING  
MEMBERS

Frederick H. Apel, Athol Springs, N. Y.

No Drawing. Application February 11, 1946,  
Serial No. 646,956

2 Claims. (Cl. 51—301)

1

This invention relates to a method of making grinding or polishing members, such as wheels or pads used for grinding or polishing plastics and softer metal, such as lead, solder, white metal, aluminum, brass and magnesium.

Heretofore such members usually comprised a plurality of layers of woven sheets of cotton cloth or felt coated with an abrasive which is unsatisfactory because the same not only became loaded with particles of metal or the like which were removed from the article being ground or polished and thus required frequent dressing and recoating to restore the grinding or polishing effect, but the same also lacked durability and required frequent recoating with abrasive in order to maintain the same in effective condition so that work of this character was unduly expensive.

It is the object of this invention to provide a method of making grinding or polishing wheels or pads which is strong, durable and flexible and well suited for doing work of this kind and incapable of becoming loaded with removed particles and also does not require dressing to maintain the same in effective condition.

The principal ingredients in the compound used in this invention and the relative quantities of the same are as follows:

|                                                                                                                                        |        |       |
|----------------------------------------------------------------------------------------------------------------------------------------|--------|-------|
| Wool capable of being felted                                                                                                           | ounces | 1/2   |
| Abrasives grains, such as crocus, tripoli, pumice, carborundum or aloxite of the requisite fineness for the respective work to be done | do     | 3 1/2 |
| Glue, preferably made from hides                                                                                                       | do     | 4     |
| Water                                                                                                                                  | do     | 5     |
| Skim milk                                                                                                                              | do     | 4 1/2 |
| Glycerine                                                                                                                              | do     | 3 1/4 |
| Borax                                                                                                                                  | grains | 40    |
| Wax, preferably ceresin                                                                                                                | drams  | 1     |
| Formaldehyde, 37% or paraformaldehyde either in liquid or powdered form                                                                | ounces | 3/8   |

If desired the following constituents in the quantities named may be included in the compound:

Drams

|                               |   |
|-------------------------------|---|
| Soap, preferably yellow chips | 1 |
| Sugar                         | 1 |

The method of mixing these ingredients and treating the same to produce the compound in accordance with this invention is as follows:

The glue is first softened by soaking the same in the water and then the same is melted at a low temperature, preferably in what is commonly known as a double boiler.

Into this melted glue the 4 ounces of milk and

2

glycerine are introduced and thoroughly mixed by stirring these several ingredients.

Thereafter 30 grains of borax are added to the above mentioned mixed and stirred ingredients 5 until this borax is thoroughly dissolved.

To this main mixture is next added a previously prepared separate mixture of ingredients consisting of the one dram of wax which has been melted at a temperature of about 150 degrees 10 Fahrenheit, 1/2 ounce of milk and the 10 grains of borax, this separate mixture being stirred into the main mixture while the combined mixtures are being heated in a boiler up to a temperature of 212 degrees F. and the stirring continued until 15 ebullition of the combined main and separate mixtures has stopped.

Stirring of this total mixture may be continued until it is of smooth consistency and spreadable like any wood worker's glue, and if the resultant 20 product is found too thick, due to evaporation, the same may be thinned to the required consistency by the addition of a suitable amount of water.

The combined mixture thus far described constitutes the binder or bonding medium with which the wool fiber and abrasive grains are now mixed so as to thoroughly coat the fibers and abrasive grains. In assembling the several ingredients of this compound the wool fiber is spread in a 25 fluffy state on a warm slab to form a sheet, the abrasive grains are spread over this sheet, and sufficient of the binding solution is poured on top of this layer to thoroughly wet the fibers and grains. Thereafter this sheet is folded several times with a broad knife to form a plurality of layers and tamped with a suitable tool to produce an even mixture and felting of the fibers. A layer of the folded mass is then placed in the 30 mold and sprayed with formaldehyde and tamped, and thereafter the other layers are successively 35 placed one on top of another in the mold and each additional layer is similarly sprayed with formaldehyde and tamped until the mold is filled. The 40 filled mold is then placed in a chamber heated to 45 about 110 degrees F. for about five hours, to cure the mass, and then the compound mass is removed from the mold and allowed to air dry from 12 to 15 hours.

When using sugar and soap as part of the compound, these ingredients are added to the mixture 50 after the introduction of the skim milk, glycerine and 30 grains of borax and stirred therewith until thoroughly dissolved.

The tamping of the mass distributes the bonding medium and the abrasive grains uniformly

throughout the mass, and also facilitates the felting of the wool fibers, and the heating of the mass at this time accelerates the action of the formaldehyde.

While being cured the mass is shaped by appropriate molds into the form of wheels, blocks, pads, rods or any other desired shape to suit the requirements of the particular work in hand.

In the foregoing compound the action of the glycerine on the glue is to keep the latter from drying out when the same is mixed with milk, borax and wax and treated under heat after formaldehyde is added to the mixture and thus forms a non-tacky and insoluble, but pliable mass which will not get brittle when subjected to a drying heat of room temperature indefinitely.

The borax also acts upon the milk, in combination with the glycerine and formaldehyde, to render the compound viscous and stable and prevent the same from crystallizing and drying out.

The presence of milk, glycerine and borax in the compound renders the same viscous and non-drying and fortifies the glue against drying out.

The wax acts as a lubricant that prevents shrinkage and stickiness under heat which is generated when utilizing a member made of this compound for grinding or polishing purposes.

By varying the glycerine, wax and water content in the compound the density of the grinding or polishing member may be varied to make the same harder or softer to suit the same for grinding or polishing plastics and metals of varying degrees of hardness.

If desired sugar and soap in the amount mentioned may be added to this composition, the sugar aiding in rendering the compound flexible and the soap preventing tackiness of the grinding or polishing member and helping to expel the detritus therefrom.

In its finished condition this compound is sufficiently friable that a grinding or polishing member made of the same will wear away and still not be excessively tough to interfere with its proper grinding and polishing function.

As a whole this compound has a high degree of pliability, elasticity and adhesiveness sufficient to reliably cement the wool fibers and abrasive grains together and retain the requisite cushion effect of the wheel or other member made of this compound.

Moreover the binding medium in this compound will not permit the detritus which is removed from the article being ground or polished to load up or cling tenaciously to the grinding or polishing member, but instead will throw off or unload such detritus from this member and maintain the working surface constantly in a clean sharp condition and thus avoid the necessity of frequent dressing of this member for maintaining the same in a high state of efficiency.

In polishing and grinding members, as heretofore constructed of solid carborundum, emery or other abrasive, the working surface of such members becomes loaded or glazed with detritus or

particles removed from the article being ground or polished by the impact of this member with said article, especially when working on softer metals and plastics.

Inasmuch as the wool fibers are intimately distributed among the sharp abrasive grains a cushioning effect is produced during impacts of the grinding or polishing member against the article being treated which has the effect of loosening the removed particles and causing the same to fall off or be thrown off the polishing or grinding member and thus automatically maintain the latter in good working condition without necessitating any dressing or cutting down operation for this purpose.

I claim as my invention:

1. The method of making a non-loading, resilient, abrasive grinding member, which comprises spreading a layer of wool in a fluffy state on a warm surface, spreading abrasive grains over said layer, applying a heat curing liquid adhesive binder to said layer and grains to thoroughly wet the same, folding said layer over, tamping said folded layer to felt said wool and incorporate said adhesive binder and grains as a homogeneous mass, filling a mold with said mass, heating said mold to cure said adhesive, and removing said mass from said mold.

2. The method of making a non-loading, resilient, abrasive grinding member, which comprises spreading a layer of wool in a fluffy state on a warm surface, spreading abrasive grains over said layer, applying an aqueous mixture of animal glue, glycerine, borax, casein and ceresin wax to said layer and grains to thoroughly wet the same, folding said layer over, tamping said folded layer to felt said wool and incorporate said aqueous mixture and grains as a homogeneous mass, applying formaldehyde to said mass, filling a mold with said mass, heating said mold to about 110° F. for about five hours to cure said aqueous mixture, and removing said mass from said mold and drying the same.

FREDERICK H. APEL.

#### REFERENCES CITED

The following references are of record in the file of this patent:

#### UNITED STATES PATENTS

| Number    | Name            | Date           |
|-----------|-----------------|----------------|
| 290,368   | Sperry          | Dec. 18, 1883  |
| 305,139   | Boynton et al.  | Sept. 16, 1884 |
| 684,710   | Olson           | Oct. 15, 1901  |
| 799,200   | Slager          | Sept. 12, 1905 |
| 1,302,320 | Damon           | Apr. 29, 1919  |
| 1,693,697 | Hafner          | Dec. 4, 1928   |
| 1,777,162 | Biddle          | Sept. 30, 1930 |
| 1,814,768 | Rippey et al.   | July 14, 1931  |
| 2,062,671 | Lupo            | Dec. 1, 1936   |
| 2,191,803 | Oesterle        | Feb. 27, 1940  |
| 2,129,377 | Libovitz et al. | Sept. 6, 1938  |
| 2,325,180 | Egeberg         | July 27, 1943  |
| 2,334,572 | Melton et al.   | Nov. 16, 1943  |